

(No Model.)

M. RANDOLPH.  
JOURNAL BEARING.

No. 349,055.

Patented Sept. 14, 1886.

*Fig. 4.*



*Fig. 1.*



*Fig. 5*



*Fig. 2.*



*Fig. 3.*



Witnesses.

W. S. Bellomy  
Eugene H. Randolph

Inventor.

Malton Randolph

# UNITED STATES PATENT OFFICE.

MAHLON RANDOLPH, OF NEW YORK, N. Y., ASSIGNOR TO THE RANDOLPH MANUFACTURING COMPANY.

## JOURNAL-BEARING.

SPECIFICATION forming part of Letters Patent No. 349,055, dated September 14, 1886.

Application filed March 26, 1886. Serial No. 196,671. (No model.)

*To all whom it may concern:*

Be it known that I, MAHLON RANDOLPH, of the city, county, and State of New York, have invented a new and useful Improvement in 5 Journal-Bearings; and I hereby declare the following to be a full and clear description thereof.

This invention relates to that class of journal-bearings or bearings for any form of moving 10 machinery in which the bearing proper is formed of an anti-friction compound, the use of which, while it forms a sufficiently hard and durable bearing, obviates the necessity of using any lubricant to reduce the frictional resistance 15 to the moving parts.

The invention will be readily understood by the subjoined specification, and by reference to the accompanying drawings, of which—

Figure 1 is a sectional elevation of the collar-bearing of a mill-spindle. Fig. 2 is a sectional elevation of the step of a mill-spindle. Fig. 3 is a plan view of the collar-bearing of the mill-spindle. Fig. 4 is an elevation of a pillar-block. Fig. 5 is an isometrical perspective view of a railway journal-bearing or similar structure.

In each of these bearings, or in any others adapted to carrying, sustaining, or guiding the moving parts of any form of machinery, the 30 bearing is formed of a retaining-case, A, usually of metallic construction, and a bearing or wearing seat, B, which is formed of my improved anti-friction compound, as described below. In most cases the shell A, whether it 35 be a spindle-collar or step-piece, a pillow-block or bearing, built in one or more pieces, or a simple journal-bearing, or any similar structure, is simply a metallic housing formed into the shape required, and adapted to receive and hold the bearing material B simply 40 by frictional contact or the cohesion produced between the parts A and B by pressing the latter, while in a plastic state, into the seat prepared for it in the former. In some cases, 45 however, this simple contact between the parts is inadequate to the purpose of holding them together, and in such cases I form one or more locking-pieces, a, on the contacting surface of the matrix-piece A, the said locking-piece a 50 in each case being formed so as to lock and

hold the material B tightly up to A, as shown by the dovetailed form in Figs. 4 and 5.

The anti-friction compound is formed of a hard and durable woody fiber, which forms the body of the working bearing, an unctuous carbonaceous matter—such as very finely-powdered graphite—which acts as a durable lubricating medium, and an adhering substance in the form of an albumen, for firmly cementing the two first-mentioned component parts into a 55 homogeneous paste, which, when thoroughly incorporated, is pressed into a mold or form, or into the required shape in the shell, when so desired.

Many former attempts to produce good and 60 durable anti-friction bearings, with plumbago or graphite as a durable lubricant, held in place by a fibrous substance and an adhering mixture, have been more or less successful; but the bearings so made have necessarily 65 been, to a certain extent, crude and unsatisfactory, by reason of the inaptitude to the purpose of the fibers used, these having been heretofore limited to such mineral substances as mineral wool, asbestos, and similar varieties of hornblende and pyroxene, and to animal hair or wool; but all such substances are adaptable to only a limited number of uses, owing to the harsh and unyielding nature of such fibers, which prevents their being pressed 70 into the finer forms of bearings, and the absence from them of sufficient firmness of substance to endure cutting or trimming after having been pressed into the desired form has rendered journal or similar bearings so formed 75 of impossible adaptation to many forms of bearings, and more or less unsuitable for all or any bearings. Another difficulty, heretofore experienced in the construction of bearings of this class, has been found in the adhering 80 substance used, such materials as liquid silicate of soda and various adhering gums having been used, each of which has shown the want of something better for the purpose, as the silicate caused the bearings to rust 85 when standing idle, and the gums being of insufficient binding or adhesive strength to produce the solidity of structure required. These difficulties have been found to be wholly met 90 and overcome in the present invention.

The woody fiber I use is taken from the hardest of woods, themselves heretofore found to form excellent journal-bearings—such woods, for instance, as box-wood, lignum-vitae, rose-wood, &c. It is usually sufficient that the wood prepared for this purpose be simply in the form of sawdust, more or less fine, in the proportion to the size of the bearing to be constructed; but in some cases, especially for very large bearings or for those required to endure great pressure, the woody fiber should be cut into splints of more considerable length. These woody particles are mixed with as much finely-powdered ("floated") graphite as will readily be taken up and bound together by the said woody fibers. To this mass I add as much strong albumen (preferably egg albumen) as the mixture will require to thoroughly cement and hold it together. The mass thus compounded is thoroughly mixed and incorporated together, so as to form a homogeneous mass. This mixing can best be done in a machine adapted to the purpose, and after the mass shall have been thoroughly incorporated together, it is put into suitable molds or formers, or into the metallic shell designed to receive it and hold it in the form of any particular bearing, and then pressure is applied, so as to make the plastic material assume an exceedingly compact form, after which it is allowed to indurate, and this may be properly hastened

by placing the said prepared bearings in a steam-heated room. After the bearings shall have become thoroughly dried and hardened in this manner, they may be faced, cut, 35 trimmed, bored, or reamed, so as to be nicely adjusted to any kind of bearing for moving machinery.

Having described my invention, I claim—

1. An improved journal-bearing or machinery-support formed of woody fiber, graphite, and albumen, combined and treated as herein described. 40

2. In a journal or other machine bearing, a constant and durable lubricant formed of an 45 unctuous carbonaceous matter, such as finely-powdered graphite, held in any prescribed form by an admixture of woody fiber and a cementing material in the form of an albumen, substantially as described.

3. A journal or other machinery bearing, formed of woody fiber in the shape of sawdust or short and small fragments of the wood mixed with finely-powdered graphite, and a cementing albumen, thoroughly incorporated 50 by mixing, then pressed into the required form, and after that thoroughly indurated by drying. 55

MAHLON RANDOLPH.

Witnesses:

J. A. J. NEAFIE,  
EUGENE H. L. RANDOLPH.